

Dec. 16, 1924.

1,519,221

E. SCHÜRER

CONTINUOUSLY LOADED CONDUCTOR

Original Filed Aug. 6, 1923

Fig. 1.



Fig. 2.

Inventor  
E. Schürer  
By Marks & Clark  
Atty.

## UNITED STATES PATENT OFFICE.

EUGEN SCHÜRER, OF COLOGNE-MULHEIM, GERMANY.

## CONTINUOUSLY-LOADED CONDUCTOR.

Original application filed August 6, 1923, Serial No. 656,135. Divided and this application filed October 21, 1924. Serial No. 745,043.

*To all whom it may concern:*

Be it known that I, EUGEN SCHÜRER, a citizen of the German Republic, and residing at Genovevastrasse 94, Cologne-Mulheim, Germany, have invented certain new and useful Improvements in and Relating to Continuously-Loaded Conductors, of which the following is a specification.

In specification Serial No. 656,135 I have described a process for producing equal values of self-inductance per unit of length of the lengths of manufacture of continuously loaded conductors, by producing such unequal values of permeability in each length by the annealing of the continuously loaded conductors that in spite of the differences in the weight of iron, all the lengths of manufacture receive the same mean value of self-inductance per unit of length. The value of the self-inductance which changes during the annealing, is measured, and the annealing is effected by passing an electric current through the continuously loaded conductor so as to be able to measure and regulate it accordingly.

It has been found that certain iron alloys which are especially suitable as loading material, because of their high permeability, must be annealed to such a high temperature and for such a short period of time for obtaining its maximum permeability, that the electric annealing process is no longer suitable therefor. In view of the fact that in this case the heat is produced in the copper from which the heating of the loading material is derived with comparatively substantial losses and moreover in view of the fact that the duration of annealing must be very short, such a high temperature has to be produced in the copper conductor above the required annealing temperature of the loading material that the latter reaches its melting limit and is destroyed. This led to the problem of thinking out an annealing process in which on the one hand the winding could be brought in a sufficient short time to the required temperature without the conducting copper being affected and in which, on the other hand, the self-inductance of the continuously loaded conductor could be measured during the annealing.

According to the invention use is made of an annealing process which is known per se as regards the annealing of wires and continuously loaded conductors, but which has

hitherto not been used in connection with the simultaneous measurement of the self-inductance.

According to this annealing process, a portion of the conductor, and not the whole length of it, is brought to the annealing temperature, a source of heat being moved along the continuously loaded conductor at a speed corresponding to the required time of annealing and imparting heat thereto from the outside, that is to say over the winding, the said source of heat being capable of bringing to the annealing temperature only a short portion of the conductor. It will thus be seen that in this way the annealing point, the temperature of which can be checked by means of a pyrometer, moves along the whole length of the conductor.

During the measurement of the self-inductance of the conductor that is effected simultaneously with the above annealing, a gradual increase in the measured value is observed during the progress of annealing. By taking into consideration the minimum value of self-inductance per unit length that is attainable with the used loading material for the greatest difference in the weight of iron, all lengths of manufacture can thus be adjusted to a constant value by interrupting the annealing when this value has been attained in each individual length of manufacture. At the utmost a short end piece of the length of manufacture remains un-annealed which accordingly shows a smaller self-inductance per unit length as compared with the annealed portion. However, this inequality has no damaging influence on the homogeneity of the conductor constituted by the individual lengths of manufacture because the length of conductor that shows this inequality is but infinitesimally small as compared with the wave lengths of the electrical waves that are propagated along the conductor. What is essential for the homogeneity of the whole of the conductor is that the value of the self-inductance per unit of length of the lengths of manufacture has the desired constant value.

As regards the measuring of the self-inductance during the annealing, the value of the self-inductance of the length of manufacture due to the winding has to be ascertained. This value is the difference between the value that has been obtained from the measurement of the continuously loaded con-

ductor and the value that has been obtained from the measurement of a similar conductor without winding in the same arrangement in space.

- 5 The measurement according to the invention is effected as follows:—Prior to the annealing, the length of manufacture is wound on a drum *i* (Fig. I) in a well defined manner for instance in the form of regular 10 spirals without the individual turns touching each other and therefrom it is passed over the annealing point *k* in a regular manner and wound on a second drum *l* and the terminals provided on the two ends of the 15 length of manufacture are connected to the measuring device *f*, for instance a Wheatstone alternating current bridge, through a sliding contact *m* provided at one end of each drum. If this measurement is carried 20 out with a conductor without winding for each position of the two drums, a value is obtained which has to be deducted from the self-inductance value of the continuously loaded conductor corresponding to the same 25 position of the two drums in order to obtain the value of the self-inductance due solely to the winding.

The following is a more simple arrangement according to the invention. The continuously loaded conductor *a* (Fig. II) is wound in regular spirals on a drum of fire-resistant material, being held away from its surface by distance pieces provided at regular intervals, which distance pieces are so 30 small that they cannot well be indicated on the drawing. During the rotation of the drum by means of the handle *n* the source of heat which according to the invention preferably consists in this case of a blast- 35 flame *o*, is moved along the longitudinal axis of the drum so that the annealing point moves along the whole length of the conductor that is wound on the drum. The connection required for the measuring 40 is again effected through the intermediary of sliding contacts *p* provided at the ends of the drums. The measuring of the self-inductance is a very simple operation 45 in this particular case since in this arrangement the formation of the conductor maintains its form during the whole annealing 50 operation.

What I claim is:—

1. A process for producing equal values 55 of self-inductance per unit of length of each length of manufacture of a continuously loaded conductor, consisting in annealing

the conductor by a source of heat that is relatively moved to the conductor, conveying the annealing heat thereto from the outside 60 and bringing each time only a comparatively short portion thereof to the annealing temperature, simultaneously measuring the self-inductance, and stopping the annealing at the moment when the desired value of the self-inductance is attained.

2. A process for producing equal values of self-inductance per unit of length of each length of manufacture of a continuously loaded conductor, consisting in winding the conductor on a drum in well defined spirals which do not touch each other, moving it therefrom in a regular manner relatively to a source of heat that is relatively moved to the conductor, conveying the annealing heat thereto from the outside and bring each time only a comparatively short portion thereof to the annealing temperature, simultaneously measuring the self-inductance, stopping the annealing at the moment when the desired value of the self-inductance is attained and winding the conductor onto a second drum.

3. A process for producing equal values of self-inductance per unit of length of each length of manufacture of a continuously loaded conductor, consisting in winding the conductor on a drum in regular spirals and annealing it by an external source of heat that is moved along the longitudinal axis 90 of the drum whilst the latter is rotated, in such a manner that the annealing point follows the whole length of the conductor that is wound on the drum, simultaneously measuring the self-inductance and stopping the annealing at the moment when the desired value of the self-inductance is attained.

4. A process for producing equal values of self-inductance per unit of length of each length of manufacture of a continuously loaded conductor, consisting in annealing the conductor by a blast-flame that is relatively moved to the conductor, the annealing heat being conveyed to the conductor from the outside and bringing each time only a comparatively short portion thereof to the annealing temperature, simultaneously measuring the self-inductance, and stopping the annealing at the moment when the desired value of the self-inductance is attained.

In testimony whereof I have signed my name to this specification.

EUGEN SCHÜRER.